

Feb. 3, 1931.

G. AURIEN

1,791,260

APPARATUS AND METHOD FOR MAKING WIRE GLASS

Filed May 7, 1929



INVENTOR  
GEORGE AURIEN  
BY  
*Cooper, Kerr & Dunham*  
HIS ATTORNEYS

## UNITED STATES PATENT OFFICE

GEORGE AURIEN, OF ST. LOUIS, MISSOURI, ASSIGNOR TO MISSISSIPPI GLASS COMPANY,  
OF NEW YORK, N. Y., A CORPORATION OF NEW YORK

## APPARATUS AND METHOD FOR MAKING WIRE GLASS

Application filed May 7, 1929. Serial No. 361,042.

This invention pertains to the manufacture of wire glass, with special reference to the placing of the wire mesh in the sheet of glass in proper position and then holding it there.

It has been customary in the manufacture of wire glass by the "two-pour" method, to first form a partially chilled sheet of glass of half the thickness of the finished sheet, then to feed the wire to lie on the upper surface of the half-sheet, and then add another layer of glass above the wire to form the finished sheet with the wire exactly in the middle thereof. One problem in this process is in keeping the wire in the middle of the glass after it has been once placed there. The difficulty arises from the fact that the wire is laid on the outer or convex side of the half-sheet before it reaches the forming pass, and then, after leaving the pass and while the upper half-sheet is still more molten than the lower half sheet, the direction of motion of the finished sheet is changed, so that the wire is on the concave side of the first half-sheet and tends to pull out through the upper half-sheet with the result that the wire in the finished sheet is displaced from its central position and a defective product results.

The object of this invention is to overcome the above difficulty by keeping the wire always on the convex surface of the first half-sheet, which is comparatively stiff, until the whole sheet has stiffened sufficiently to prevent movement of the wire.

Further and other objects and advantages will be apparent from the specification and claims, and from the accompanying drawings which show by way of illustration what is now considered to be the preferred form of the invention.

The drawing is a somewhat diagrammatic cross-section of a sheet glass rolling machine arranged to roll wire glass by the two-pour process.

Molten metal 10 flows from the furnace at the left between lower roll 12 and upper roll 14 to form the first half-sheet 16, which is half the thickness of the finished sheet. This half-sheet is carried on roll 12 toward side

roll 18, which is set to form a sheet double the thickness of the half-sheet 16. While on roll 12, sheet 16 is partially stiffened by contact on its lower side with the roll and on its upper side with the air. While in this partially stiffened condition, the wire mesh 20 is fed over rollers 22 and 24 onto the upper surface of sheet 16, and immediately thereafter sheet 16, with the wire on its upper surface, passes into and through molten metal 26, which flows from the right, to the pass between rollers 12 and 18, where the finished sheet is formed, the wire being in the middle of that sheet, between the convex surface of sheet 16 and the concave surface of the newly formed and comparatively molten half-sheet.

After leaving the lower pass, it is customary to direct the finished sheet to the right of apron 30 and over rolls 32 to the leer. This change of direction puts the wire on the convex side of the newly formed half-sheet, with the result that the wire being under some tension tends to become displaced from its former resting place on half-sheet 16 to some indefinite position in the newly formed and comparatively molten half-sheet, where it remains.

According to the present invention, the completed sheet passes to the left of apron 30 and is guided close to roll 12 until the sheet is cooled and stiffened sufficiently to prevent displacement of the wire, whereupon the sheet passes into the leer over rolls 34. In this manner the wire is always maintained against the convex surface of the stiffened half-sheet 16, with the result that the wire is not displaced but remains central in the finished sheet.

It is to be understood that the invention is not limited to the specific embodiment and construction herein specified but may be used in other ways without departure from its spirit as defined by the following claims.

I claim—

1. In the process of forming wire glass, the steps of forming a first half-sheet, slightly stiffening said half-sheet by contact with a cooling roller, placing wire mesh on the convex surface of said stiffened half-sheet, form-

ing the finished sheet by adding another half-sheet to the outer surface of the first half-sheet whereby the wire is in the middle of the sheet, and thereafter so guiding said sheet  
5 that the convex surface of the first half-sheet is continually presented to the wire until the sheet is sufficiently chilled to prevent the wire from leaving its original position in the sheet.

10 2. In a machine for forming wire glass, in combination, a pair of rolls forming a pass therebetween for forming a first half-sheet, means comprising one of said rolls for conducting said half-sheet from said pass,  
15 whereby said half-sheet is slightly stiffened, means for placing wire mesh on the convex surface of said stiffened half-sheet, and means comprising rolls forming a second roll pass for forming the finished sheet by adding another half-sheet outside of said wire, and  
20 means comprising a concave apron for subsequently guiding said sheet to the leer, said guiding means acting to maintain the wire on the convex surface of the first half-sheet  
25 until the sheet is sufficiently stiffened to prevent displacement of the wire from its central position in the sheet.

In testimony whereof I hereto affix my  
signature.